

1,586,877

June 1, 1926.

O. E. BUCKLEY

ELECTROMAGNETIC DEVICE

Filed April 4, 1924

2 Sheets-Sheet 1

Fig. 1.



Fig. 2.



Fig. 4.



Inventor:  
Oliver E. Buckley  
by *Low Adams Atty.*

June 1, 1926.

1,586,877

O. E. BUCKLEY

ELECTROMAGNETIC DEVICE

Filed April 4, 1924

2 Sheets-Sheet 2

Fig. 5.



Inventor:  
Oliver E. Buckley  
by *John W. Adams - Atty.*

Patented June 1, 1926.

1,586,877

# UNITED STATES PATENT OFFICE.

OLIVER E. BUCKLEY, OF MAPLEWOOD, NEW JERSEY, ASSIGNEE TO WESTERN ELECTRIC COMPANY, INCORPORATED, OF NEW YORK, N. Y., A CORPORATION OF NEW YORK.

## ELECTROMAGNETIC DEVICE.

Application filed April 4, 1924. Serial No. 704,127.

This invention relates to electromagnetic structures and in particular to such structures making use of a magnetic member of nickel-iron alloy having high permeability and low hysteresis loss.

It is an object of the invention to decrease the hysteresis loss and to maintain high permeability in certain magnetic alloys in which high permeability may be developed. Other objects of the invention will appear from the following disclosure.

To attain the above mentioned object, and in accordance with the preferred embodiment of the invention, there is provided a core or member of magnetic material for an electric coil or circuit, which material consists of or comprises an alloy of nickel and iron in the proportions of 78½% nickel and 21½% iron, and the magnetic member is subjected to a constant tension during operation.

It has recently been found that a nickel-iron alloy of the proportions just mentioned, when properly heat treated, has remarkably high permeability at low magnetizing forces coupled with high resistivity and low hysteresis loss. So marked are the desirable characteristics of this material that it has already found wide and important applications in the electromagnetic arts. Whereas the permeability of iron at low magnetizing forces is around 300, that of the new material is ordinarily from ten to twenty times as great and may be made still greater by careful treatment. The hysteresis loss per cubic centimeter per loop for which the limiting value of the induction is 5,000 c. g. s. units is around 200 ergs or less. By "low" magnetizing forces is meant those much less than a gauss. The highest permeability of the new material ordinarily is reached when the force is a small fraction of a gauss. These are the forces encountered in signaling so that this material is particularly valuable in the signaling field. The name permalloy has been applied to this and similar nickel-iron alloys. For a more complete description of these alloys see U. S. application of G. W. Elmen, Serial No. 473, 877, filed May 31, 1921.

It has now been discovered that when such a nickel-iron alloy has been suitably heat treated and then placed under tension of the proper amount there is produced in it the following advantageous changes.

The permeability at a low field strength increases to a point where it becomes relatively stable with respect to the tension over a certain range and the coercive force and hysteresis loss fall to an almost negligible value—in certain instances to less than one quarter that of the same material when not strained. Furthermore, portions of the B—H curve become very straight and the change in permeability near the saturation point becomes very abrupt. There is described below, a practical application of this discovery. Many other applications are, of course, possible.

In the accompanying drawing, Fig. 1 shows one embodiment of this invention in the form of a transformer having a core of the above mentioned nickel-iron alloy under constant tension; Fig. 2 is a plan view of the core of Fig. 1 with a portion broken away; and Figs. 3 and 4 are explanatory curves.

Referring to Figs. 1 and 2 of the drawing which illustrate a schematic representation to show the principles involved, there is provided a framework 1, from the top of which is suspended a magnetic coil structure 2. This coil structure comprises a primary winding 3, a secondary winding 4 and a tertiary winding 5 upon the core 6. The core 6 is of nickel-iron alloy in the form of fine wires which may be, for example, five mils in diameter. These are assembled in parallel relation to form a cylindrical mass clamped at the extremities by clamping caps 7 and 8. The upper clamping cap 7 is attached to the upper portion of the framework 1, while to the lower clamping cap 8 is attached a spring dynamometer. The movable end of the spring of the dynamometer is attached by means of a wire or cord to a shaft 9 upon which it may be wound by handle 10. Ratchet 11 and pawl 12 hold the shaft 9 in position with a desired tension applied to the core 6. Fig. 2 is a top view of the core with a portion of the cap 7 removed disclosing the upper ends of the wires forming the core. A source 13 of alternating current is connected to the primary winding 3. Source 13 represents any source of alternating current either sinusoidal or of more complex form, such as would be produced for example, by a microphone and an alternating current generator working into the same circuit. A source of

5 direct potential 14 is in circuit associated with the transformer tertiary winding 5 through variable resistance 15 and switch 16. The secondary winding 4 of the transformer is associated with any electrical translating device 17 to which it is desired to supply current.

10 The relationship of tension to permeability of the nickel-iron alloy herein described and also of iron is shown in the curves of Fig. 3, which give the results of experiments on wires of each material 0.040 inch diameter and 22 inches long. Similar results are obtainable with samples of other 15 shapes and dimensions. It will be noted that when the tension on the permalloy is zero (point *a* on the curve) the permeability is very high, relative to that of iron at an applied field strength of 0.01 gauss. 20 When a tension of 5,500 pounds per square inch is applied, to the permalloy, the permeability is thereby increased to a value of approximately 75,000, as indicated at *b*. Furthermore within the range from 5,000 25 pounds per square inch to 6,000 pounds per square inch, there is relatively little change in permeability. Iron, on the other hand, has a relatively small value of permeability which is much less affected by tension.

30 In Fig. 4 is disclosed the relationship of magnetizing force *H* to induction *B*, in the form of hysteresis loops of strained and unstrained permalloy respectively. The hysteresis loss is seen to be very much less for 35 strained than for unstrained permalloy. The width of the loop for iron (not shown) is at least one hundred times that for the permalloy under tension. Moreover the major portion of the curve for strained permalloy is remarkably straight and there is a very abrupt change in permeability at the beginning of the horizontal portions. These characteristics of the *B*-*H* curve can be utilized to advantage in various electromagnetic devices. Applicant has then discovered means for obtaining these desirable characteristics to a degree hitherto unknown.

40 To obtain the above mentioned properties in the nickel-iron alloy containing 78½% nickel, a special heat treatment is required. In a particular instance in which the desired effects were obtained, nickel-iron wire having the desired proportions of the ingredients was heated in a vacuum at a temperature of 1,100° C. for one hour. It was then allowed to cool to a temperature of 850° C. in 45 minutes, and from this temperature to room temperature in 45 minutes. 45 The correct time for heating and the rate of cooling will vary somewhat with the dimensions of the element under treatment, but can be determined by trial in each case.

50 The relation of permeability to tension for any particular iron-nickel alloy of the

approximate composition of the one here described has been found to depend greatly on the heat treatment. For instance it has been found that a wire of 78½% nickel and 21½% iron which has been mechanically 50 worked and then annealed at a temperature of 800° C. for a few minutes and allowed to cool in air will show rapid decrease of permeability with tension when measured with a field strength of .01 gauss, whereas 55 a similar wire heat treated at 1,100° C. as above described and measured with the same field strength shows a tremendous increase of permeability with tension. As pointed out in the copending application of O. E. Buckley, Serial No. 13501, filed March 6, 1925, the iron alloys of less than about 80% nickel show, when suitably heat treated, an 60 increase of permeability with tension. The 78½% alloy here described is taken as 65 representative of this class. Both the heat-treatment and the optimum tension will vary somewhat for different alloys. They can best be determined by trial in each case.

70 In the operation of the device described above, the adjustment will depend upon the purpose to be effected. If it is desired to step up or step down voltage from source 13, to supply translating device 17 without distortion, the potential from source 13 is 75 so chosen as not to cause saturation of the core 5. Voltage and current transformation is then effected with great efficiency and with substantially no loss due to hysteresis. Where the impressed current has components of different frequency the magnetic 80 modulation and flutter effects are small. Since the core is made up of small wires, the eddy current loss is likewise kept very 85 low, the resistivity of the material being 100 relatively high. The diameter of the individual wires is chosen with a view to controlling eddy current loss. The permeability is so high that a core many times 105 smaller than if the material were iron may 110 be used. In certain cases the size of the core may be reduced to a fiftieth of that required when iron is used. Since the core 115 may be small, the structure required to introduce the necessary tension may likewise 120 be small. It is thus seen that from all points of view this nickel-iron alloy is remarkably well adapted for the purposes herein described.

125 It is often desirable to close switch 16 and adjust resistance 15 to such value that the field set up by tertiary coil 5 just neutralizes the effect of the earth's field or other disturbing field. If stray field effects are large it is advisable to enclose the coil in a magnetic shield.

130 If it is desired to employ this transformer for the purpose of producing distortion, it is only necessary to choose such operating values of superposed uniform magnetic field 135

produced by battery 14 that the magnetizing force required to saturate the core will be exceeded during each cycle. In this way, modulation, detection, harmonic generation and other forms of distortion may be effected.

While a two-coil transformer is disclosed, it is obvious that an auto-transformer would operate upon the same principle and that the transformation ratio of the primary and secondary of such auto-transformer may, in a limiting case, be unity. It is obvious, also that the translating device 17 could be transferred from the secondary to the primary circuit if distortion rather than voltage or current transformation is desired.

By varying the relation between the diameter and the length of the core in a well known manner, the range of externally applied field over which the permeability remains substantially constant, may be varied at will, but, in each case, the hysteresis loss which is represented by the area of the hysteresis loop remains small.

25 What is claimed is:—

1. An electromagnetic structure comprising an electric circuit, a magnetic element in inductive relation thereto comprising an alloy of nickel and iron, and means for maintaining a constant tension in said magnetic element of such value that the permeability is greater than if no tension were applied.

2. An electromagnetic structure comprising an electric circuit, a magnetic element in inductive relation thereto comprising an alloy of nickel and iron, and means for maintaining a tension in said magnetic element of such value that the permeability is high and relatively constant for a considerable range of tension.

3. An electromagnetic device comprising an electric winding and a core therefor of magnetic material comprising an alloy of nickel and iron which has high permeability of substantially constant value over a considerable range of tensile forces, and means for applying a substantially constant tensile force within said range.

4. An electromagnetic device comprising

an electric winding and a core therefor comprising a nickel-iron alloy in the form of elements of small cross sectional area, and means for applying tension to each of said elements.

55

5. The combination with a member of magnetic material comprising nickel and iron which when placed under tension of a certain range of values increases in permeability and at the same time decreases in hysteresis loss, with means for maintaining said member under constant tension within said range.

6. A magnetic element consisting of an alloy in which nickel constitutes about 78% and iron about 22%, and means for maintaining said element under tension.

7. A magnetic element which abruptly approaches saturation at a few tenths of a gauss field strength consisting of an alloy comprising nickel and iron continuously externally strained in the direction of the flux.

8. A magnetic element, the flux of which varies substantially linearly with variations in field strength from near zero value to a value at which the material approaches saturation consisting of an alloy comprising nickel and iron continuously externally strained in the direction of the flux.

9. A magnetic element having a coercivity of the order of a hundredth that of iron consisting of an alloy comprising nickel and iron continuously externally strained in the direction of the flux.

10. A magnetic material having high permeability at low magnetizing forces in combination with means for applying an elongating stress to the material whereby its permeability at low magnetizing forces is increased and its hysteresis loss decreased.

90

11. A magnetic element consisting of an alloy in which nickel constitutes about 78% and iron about 22%, and means for maintaining said element under a constant tension of approximately 5,500 pounds per square inch whereby the coercivity of the material is substantially lowered.

95

In witness whereof, I hereunto subscribe my name this 3 day of April A. D., 1924.

OLIVER E. BUCKLEY.